

## UNITED STATES PATENT OFFICE.

FRITZ HARTNER, OF HOMBURG, GERMANY.

## PROCESS FOR MANUFACTURING A MORTAR-FORMING MATERIAL FROM ANHYDRITE.

No Drawing. Application filed November 12, 1920. Serial No. 423,762.

*To all whom it may concern:*

Be it known that I, FRITZ HARTNER, superintendent, a subject of the German State, residing at Homburg v. d. Hohe, State of Prussia, Germany, have invented certain new and useful Improvements in Processes for Manufacturing a Mortar-Forming Material from Anhydrite, of which the following is a specification.

10 Hitherto anhydrite could not be turned into a mortar-forming material having suitable self-setting properties. Only recently means have been proposed directly allowing the use of anhydrite for mortar-preparation, 15 with or without the addition of other ingredients. Now I have been successful in obtaining a mortar-forming-agent by the mere use of anhydrite, with no other means for attaining the setting properties.

20 A quite surprising solution of the problem consists in grinding the anhydrite as fine as it can possibly be done. When it is pulverized in suitable grinding apparatus to its fullest extent, it sets without any further 25 additions and without any further treatment, having the hardening power of an efficient mortar-forming material.

The speed of setting will be all the quicker and the figures of resistance will be the 30 more favourable, the more impalpable the pulverization.

The essential feature of the invention is thus the ascertaining that anhydrite, not capable of setting of itself, or sulphate of calcium in a similar state or anhydrite-bearing rock may be converted into a mortar-forming material, if the grinding process is pushed to a sufficient degree.

35 Trials have evinced that anhydrite, resulting in a residue of from 20 to 30% on the 900 meshes sieve, is still fully inert, but shows thorough setting and satisfactory

hardening power when ground so as to have greatest possible amount of fine powder, 45 passing through a 10,000 mesh per sq. cm. sieve, i. e., powder below 0,006 mm. in size.

For putting in practice this kind of the new process, anhydrite or the anhydrite-bearing rock has to be powdered with such 50 grinding apparatus that the proper portion of fine powder or, in more precise terms the impalpable dust like powder is as great as possible. Either such grinding mechanisms as, e. g., ball- and tube-mills, are to be selected which immediately provide the required 55 degrees of impalpability in a sufficiently extended period of grinding or else the grinding contrivances are to be so devised or to be so conducted that principally a fine powder is obtained.

For the purpose are recommended by preference the mills operating with balls as pulverizing media, such as pebbles or steel-balls. As an example of such mills I may mention in addition to the ball- or drum-mills proper, 65 tube-mills, compound-mills, horizontal ball-mills. The required impalpability i. e. the prevailing of the finest powder in the dust like product is obtained the more reliably as the grinding surface is longer.

70 I claim:

1. A self-setting anhydrite mortar forming material of a fineness passing through a screen of 900 mesh per square cm.

2. A self-setting anhydrite mortar material the major portion of the particles of which will pass through a screen of 10,000 mesh per sq. cm.

75 In testimony whereof I affix my signature in presence of two witnesses.

FRITZ HARTNER.

Witnesses:

WILLY HARTNER.

JOHANNA HARTNER.